

## UNITED STATES PATENT OFFICE

2,159,723

## APPARATUS SUBJECTED TO HEAT AND COLD ALTERNATELY

Russell Franks, Niagara Falls, N. Y., assignor to Union Carbide and Carbon Corporation, a corporation of New York

No Drawing. Original application June 18, 1935, Serial No. 27,161. Divided and this application April 27, 1937, Serial No. 139,258

2 Claims. (Cl. 75—126)

The invention relates to apparatus and parts thereof which during use are alternately heated to temperatures above about 200° C. and cooled to temperatures in the neighborhood of 0° C. or lower, and it is the principal object of the invention to provide alloy steel apparatus and parts which under such conditions of use retain toughness and resistance to impact. This application is a division of my application Serial No. 27,161 filed June 18, 1935.

Numerous manufacturing processes, notably oil refining, employ pressure vessels and machine elements at elevated temperatures, and not uncommonly this apparatus is subjected from time to time to zero or subzero temperatures, either by intentional refrigeration or by cold weather. Apparatus for use at high temperatures, particularly in the presence of corrosive conditions, is frequently constructed from steel containing substantial amounts of chromium. Except in situations wherein the corrosive conditions are unusually severe, ferritic steel containing about 4% to 10% chromium is usually chosen as the most economical material. A small amount of molybdenum or tungsten is sometimes added to increase the strength and toughness of this steel at elevated temperatures.

It has been observed that the above described steel, after prolonged exposure to high temperatures, tends to lose a great part of its resistance to impact at low temperatures, and equipment subjected alternately to very high and very low temperatures has frequently failed by cracking. Steel containing molybdenum or tungsten appears to be almost as susceptible to this type of failures as the steel containing no molybdenum or tungsten.

Another difficulty encountered in the fabrication and use of this steel is its ability to harden and become brittle when rapidly cooled from high temperatures. This property increases considerably the difficulties in designing, fabricating, and operating corrosion resisting equipment.

The addition of suitable amounts of titanium or columbium, or both, decreases the air-hardenability of the ferritic chromium steels, and with a proper choice of composition the material may be made substantially non-hardenable by heat treatment. But the addition of these elements, alone, does not eliminate the above discussed loss of impact strength at subzero temperatures.

I have discovered that properly proportioned additions of columbium, together with molybdenum, tungsten, or mixtures of molybdenum

and tungsten greatly improve the impact strengths of ferritic chromium steels at subzero temperatures after prolonged holding at elevated temperatures. Incidental, but by no means inconsequential, benefits imparted by these additions include a decrease in air-hardenability and an increase in resistance to corrosion and high-temperature oxidation.

Table A presents representative results of comparative tests which comprised holding wrought steel impact specimens at about 750° C. for four hours and then cooling them in air (a suitable annealing treatment); subsequently holding them at about 475° C. for one month and then slowly cooling them in the furnace; and finally holding them for three hours at —40° C., at which temperature they were subjected to a standard Izod impact test on a machine having an initial energy level of 129 foot-pounds.

Table A

| Analysis   |           |            |            |          | Izod impact |
|------------|-----------|------------|------------|----------|-------------|
| Percent Cr | Percent C | Percent Mo | Percent Cb |          |             |
| 5.87       | .06       | None       | None       | Ft. lbs. | 33          |
| 5.95       | .10       | 0.55       | None       |          | 46          |
| 6.41       | .06       | None       | 0.75       |          | 61          |
| 6.45       | .06       | 0.50       | 0.65       |          | 109         |

Results which are similar, although showing less marked differences, have been obtained in tests alternately at about 300° C. and about 0° C.

Table B shows the results of comparative tests wherein wrought steel samples were heated at about 900° C. for ten minutes, cooled in the air, and tested at room temperatures.

Table B

| Analysis   |           |            |            |          | Izod impact | Brinell hardness |
|------------|-----------|------------|------------|----------|-------------|------------------|
| Percent Cr | Percent C | Percent Mo | Percent Cb |          |             |                  |
| 5.87       | .06       | None       | None       | Ft. lbs. | 29          | 302              |
| 5.95       | .10       | 0.55       | None       |          | 23          | 340              |
| 6.41       | .06       | None       | 0.75       |          | 119         | 131              |
| 6.45       | .06       | 0.50       | .65        |          | 112         | 112              |

For the purposes of comparison with Tables A and B, Table C sets forth the properties of the steels in question, at room temperature, after annealing at 750° C. for four hours and air-cool-

5

10

15

20

25

30

35

40

45

50

55

ing (heat treatment S); and after annealing, subsequent holding at 475° C. for one month, and then air-cooling (heat treatment L).

5

Table C

| 10 | Analysis   |           |            |            | Heat treatment | Izod impact | Brinell hardness |
|----|------------|-----------|------------|------------|----------------|-------------|------------------|
|    | Percent Cr | Percent C | Percent Mo | Percent Cb |                |             |                  |
| 10 | 5.87       | 0.06      | None       | None       | S              | 108         | 126              |
|    | 5.95       | .10       | 0.55       | None       | L              | 100         | 121              |
| 15 | 6.41       | .06       | None       | 0.75       | S              | 112         | 140              |
|    | 6.45       | .06       | 0.50       | .65        | L              | 104         | 156              |
| 20 |            |           |            |            | S              | 106         | 131              |
|    |            |           |            |            | L              | 99          | 112              |
| 25 |            |           |            |            | S              | 108         | 121              |
|    |            |           |            |            | L              | 108         | 121              |

The data in Tables A, B, and C are self-explanatory and indicate the improvements provided by the present invention.

The invention comprises apparatus and parts thereof which during use are alternately heated to temperatures upwards of about 200° C. and cooled to temperatures substantially at or below about 0° C., and which consist of a ferritic alloy steel containing about 4% to 10% chromium; carbon in amounts not over 0.15%; about 0.25% to 1.5% tungsten, molybdenum, or mixtures thereof; columbium in an amount between 6 and 16 times the carbon content; not over about 0.75% silicon; the usual fractional percentages of manganese required in steel making practice; and the remainder substantially all iron. In making steels commercially, the lowest practical

percentage of carbon is in the neighborhood of 0.01%. Therefore, in the steels of the present invention, the lowest practical percentage of columbium is about 0.06%.

The most extensive use of the invention will probably be in the form of tubes for use in handling hot fluids, for instance in the pyrolysis of hydrocarbons, where the temperature during periods of heating will be upwards of 400° C.

5  
10  
15  
20  
25  
30  
35

I claim:

1. Apparatus and parts thereof which during use are alternately heated to temperatures upwards of about 400° C., cooled to temperatures at or below about 0° C. and subjected to impact stresses at the lower temperatures and which consists of a ferritic alloy steel containing about 4% to 10% chromium; 0.01% to 0.15% carbon; silicon in amounts not over about 0.75%; about 0.25% to 1.5% molybdenum; 0.06% to 2.4% columbium, the columbium content being 6 to 16 times the carbon content; the remainder substantially all iron.

2. Apparatus and parts thereof which during use are alternately heated to temperatures upwards of about 200° C., cooled to temperatures at or below about 0° C. and subjected to impact stresses at the lower temperatures and which consists of a ferritic alloy steel containing about 4% to 10% chromium; 0.01% to 0.15% carbon; silicon in amounts not over about 0.75%; about 0.25% to 1.5% molybdenum; 0.06% to 2.4% columbium, the columbium content being 6 to 16 times the carbon content; the remainder substantially all iron.

RUSSELL FRANKS. 35